

## UNITED STATES PATENT OFFICE

2,342,230

## CLOTHS FOR ELECTROCHEMICAL DIAPHRAGMS AND METHOD OF PREPARING SAME

Karl Weber and Georg Bode, Gersthofen, near Augsburg, Germany; vested in the Alien Property Custodian

No Drawing. Application July 22, 1940, Serial No. 346,872. In Germany July 21, 1939

5 Claims. (Cl. 204—296)

(Granted under the provisions of sec. 14, act of March 2, 1927; 357 O. G. 5)

The present invention relates to cloths for electrochemical diaphragms.

Various processes are already known for using filter cloths which consist of after-chlorinated polyvinyl chloride as diaphragms for electrochemical purposes. It has, however, been found that in the presence of a strongly acid electrolyte of an oxidizing action the tissue is not sufficiently tight so that even after shrinkage of the fiber in hot water of 90° C. the diffusion between the anode liquid and the cathode liquid is not prevented.

Now we have found, and this is surprising, that felt or tissue of fibers from after-chlorinated polyvinyl chloride possess the desired impermeability which have been impregnated with silicic acid and at least one water-insoluble inorganic salt. Insoluble salts of calcium and barium are particularly suitable for that purpose. The impregnation may, for instance, be produced by saturating the felt or tissue with aqueous solutions of salts of silicic acid and with metal salts, for instance barium salts and after-treating them with dilute sulfuric acid.

The after-chlorinated polyvinyl chloride is for instance obtained according to the process described in U. S. Patent No. 1,982,765.

The following examples serve to illustrate the invention, but they are not intended to limit it thereto, the parts being by weight:

(1) After-chlorinated polyvinyl chloride (for instance felt 300/2) is placed for 2 minutes into hot water of 90° C. After drying the shrank cloth is coated with an intimate mixture of 2 parts of barium sulfate and 1 part of waterglass (commercial) and allowed to dry in the open air. The cloth is then treated with sulfuric acid of about 10 per cent strength and again dried in the open air; the diaphragm is then ready for use.

(2) After-chlorinated polyvinyl chloride (for instance felt 300/2) is placed for 2 minutes into hot water of 90° C. The shrank cloth is impregnated with a barium chloride solution which has been saturated in the hot condition. The cloth is then allowed to drop off and treated with dilute sulfuric acid for causing the barium sulfate to precipitate. After drying the cloth is soaked with waterglass and the silicic acid is set free by means of dilute sulfuric acid. After having been dried in the open air the diaphragm is ready for use.

(3) After-chlorinated polyvinyl chloride (for instance felt 300/2) is placed for 2 minutes into hot water of 90° C. The shrank cloth is impregnated with calcium chloride solution and calcium phosphate is precipitated on the fiber by means of tri-sodium phosphate. The cloth is washed for a short time with water for removing the sodium chloride; it is then soaked with

commercial waterglass and the silicic acid is set free with phosphoric acid. After having washed it with water and subsequently dried in the open-air the diaphragm is ready for use.

5 We claim:

1. Filter cloths for electrochemical diaphragms which are tight in the presence of strongly acid electrolytes of an oxidizing action consisting of shrunk felted fibers of after-chlorinated polyvinyl chloride impregnated with silicic acid and at least one water-insoluble salt of a metal of the group consisting of calcium and barium.

2. Filter cloths for electrochemical diaphragms which are tight in the presence of strongly acid electrolytes of an oxidizing action consisting of shrunk felted fibers of after-chlorinated polyvinyl chloride impregnated with silicic acid and barium sulfate.

3. Filter cloths for electrochemical diaphragms which are tight in the presence of strongly acid electrolytes of an oxidizing action consisting of shrunk felted fibers of after-chlorinated polyvinyl chloride impregnated with silicic acid and calcium phosphate.

20 4. A process for producing filter cloths for electrochemical diaphragms that are tight in strongly acid electrolytes of an oxidizing action which comprises subjecting to shrinkage felted fibers consisting of after-chlorinated polyvinyl chloride and impregnating the shrank fibers with a water insoluble salt of a metal selected from the class consisting of barium and calcium and with an aqueous solution of an alkali metal silicate and freeing silicic acid from the silicate by 25 treating the impregnated cloth with an acid having an anion corresponding to the anion of said water insoluble salt.

5. A process for producing filter cloths and electrochemical diaphragms that are tight in

40 strongly acid electrolytes of an oxidizing action which comprises subjecting to shrinkage fibers consisting of after-chlorinated polyvinyl chloride, impregnating the shrank fibers with a water soluble salt of a metal selected from the class consisting of barium and calcium, treating the thus 45 impregnated cloth with an aqueous solution of a compound having an anion adapted to form a water insoluble salt with the aforementioned water soluble salt to thereby produce in said fibers an impregnation of a water insoluble salt of a metal selected from the class consisting of barium and calcium, impregnating the thus obtained cloth

50 with an aqueous solution of an alkali metal silicate and thereafter treating said cloth with an acid having an anion corresponding to the anion of said water insoluble salt to thereby free silicic acid from the silicate.

KARL WEBER.  
GEORG BODE.